

Nov. 13, 1928.

1,691,734

R. E. OBER

PEAT FUEL

Filed Aug. 15, 1927



Fig. 1.



Fig. 2.

Inventor

R. E. Ober.

By

Geo. Stevens.  
Attorney

# UNITED STATES PATENT OFFICE.

RAYMOND E. OBER, OF CROSBY, MINNESOTA.

## PEAT FUEL.

Application filed August 15, 1927. Serial No. 212,937.

This invention relates to peat fuel and has special reference to a novel form of unit of such fuel, the object of which will be described later.

5 Referring to the accompanying drawing forming part of this application and wherein like references indicate like parts:

Figure 1 is a perspective view of a unit of fuel having the advantages hereinafter described when initially formed; and

10 Figure 2 is a like view of an ultimate unit of such fuel.

From my experiments in the manufacture of peat fuel it has been determined that the 15 rate of evaporation from machined peat depends upon the surface contact with volume of air. Given a certain volume of peat, whether in a block, sheet, or other form, the greater the surface exposure the more 20 rapid the evaporation of the contained moisture. It has been found that a hollow cylinder at once gives strength of cross section and a maximum surface exposure. The ratio between surface area and volume depends on 25 thickness of the wall of the hollow cylinder. In experiments for the manufacture of peat fuel, standard pug and auger machines were used to macerate and knead raw material and shape it into a hollow column, which passed 30 over a standard taut wire cutting table which cut the column into blocks of the desired length. It was found that the speed of flow of column was limited through any size of orifice, and that volume production could be 35 attained only by increasing the size of ori-

fice in front head of auger. However, regardless of size of block, if rapid evaporation were to be obtained, a minimum thickness of wall must be had. A large block with a thin wall made of 65% to 67% moisture peat 40 is so unstable as to prevent handling. Hence a design was developed for multiple lobe small block, in which the desired ratio between surface area and volume may be maintained by the regulation of size of central 45 cores, and at the same time volume production attained, due to increase in size of cross section area of orifice.

The preferred ratio has been found to be approximately two of surface area to one of 50 volume, and any hollow cylinder irrespective of diameter having a wall one inch thick gives this desired ratio.

Having thus described my invention, what I claim and desire to secure by Letters Patent, is:

1. A unit of peat fuel initially in substantially the form of multiple hollow cylinders.
2. A unit of peat fuel initially in substantially the form of a plurality of weakly united cylinders.
3. A unit of peat fuel in substantially the form of a plurality of attached hollow cylinders, there being an axial hole therethrough for the purpose described.
4. A hollow substantially cylindrically shaped unit of peat fuel.

In testimony whereof I affix my signature.

RAYMOND E. OBER.